

## UNITED STATES PATENT OFFICE

2,311,428

## PHOTOGRAPHIC DEVELOPER

William H. Wood, Bedford, Ohio, assignor to  
 Harris-Seybold-Potter Company, Cleveland,  
 Ohio, a corporation of Ohio

No Drawing. Application December 6, 1939,  
 Serial No. 307,866

10 Claims.

(Cl. 95-88)

This invention relates to photography, and more particularly developers; and it is among the objects of the invention to improve developing procedure and compositions, and more particularly facilitate development of the so-called "fine grain" character.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

In accordance with my invention, a developing composition is made up to include piperazine and a silver halide developing agent. The piperazine may be in convenient or desired form, either anhydrous or crystalline, the latter form being more generally preferable on account of its very ready solubility, and I especially prefer the hexahydrate on account of its general availability and ease of handling. The proportions of piperazine in the developer may be varied, depending upon particular conditions. I have found in general satisfactory concentrations in the range of 0.5 to 5.0 per cent in the solution. The piperazine may be used in conjunction with various developing agents with resultant advantages, and it is particularly advantageous in fine grain developer compositions.

As an example, for fine grain developer work, the following is given:

|                        |        |      |
|------------------------|--------|------|
| Piperazine hexahydrate | grams  | 10   |
| Paraphenylenediamine   | do     | 16   |
| Glycine                | do     | 15   |
| Sodium sulphite        | do     | 90   |
| Potassium bromide      | do     | 0.33 |
| Water                  | liters | 1.2  |

The developing is carried out at customary developing temperature, usually around 70 or 75° F., but the composition is not critical as to temperature.

Also the present compounds are particularly advantageous with one or more of the amino-hydroxy compounds described in my co-pending application Serial No. 307,865, viz. an alkyl substituted amino-hydroxy aliphatic compound

sufficiently soluble for working concentration. Presence of a sulphite radical is also desirable.

As an illustrative example, the following is given:

|    |                         |        |     |
|----|-------------------------|--------|-----|
| 5  | Piperazine hexahydrate  | grams  | 10  |
|    | Paraphenylenediamine    | do     | 16  |
|    | Glycine                 | do     | 15  |
|    | Sodium sulphite         | do     | 90  |
| 10 | Trimethylolaminomethane | do     | 2.5 |
|    | Potassium bromide       | do     | 0.3 |
|    | Water                   | liters | 1.2 |

Other modes of applying the principle of the invention may be employed, change being made as regards the details described, provided the features stated in any of the following claims, or the equivalent of such, be employed.

I therefore particularly point out and distinctly claim as my invention:

- 20 In preparing photographic images, developing the image in the presence of piperazine, glycine, paraphenylenediamine, sodium sulphite and potassium bromide.
- 25 In preparing photographic images, developing the image in the presence of piperazine, an aliphatic amino compound of the general formula



30 in which R is an alkyl radical and R' is an alkyl which optionally may have a hydroxyl sufficiently soluble for working concentration, a compound providing a sulphite radical, and a silver halide developing agent of fine grain type.

- 35 In preparing photographic images, developing the image in the presence of piperazine, an aliphatic amino compound of the general formula



45 in which R is an alkyl radical and R' is an alkyl which optionally may have a hydroxyl sufficiently soluble for working concentration, and a silver halide developing agent.

- 50 In preparing photographic images, developing the image in the presence of piperazine

0.5 to 5.0 per cent and a silver halide developing agent of fine grain type.

5. In preparing photographic images, developing the image in the presence of piperazine 0.5 to 5.0 per cent and a silver halide developing agent.

6. A photographic developer containing piperazine, glycine, paraphenylenediamine, sodium sulphite and potassium bromide.

7. A photographic developer containing piperazine, an aliphatic amino compound of the general formula



in which R is an alkyl radical and R' is an alkyl which optionally may have a hydroxyl sufficiently soluble for working concentration, a compound providing a sulphite radical, and a silver halide developing agent of fine grain type.

8. A photographic developer containing piperazine, an aliphatic amino compound of the general formula



in which R is an alkyl radical and R' is an alkyl which optionally may have a hydroxyl sufficiently soluble for working concentration, and a silver halide developing agent.

9. A photographic developer containing piperazine 0.5 to 5.0 per cent and a silver halide developing agent of fine grain type.

10. A photographic developer containing piperazine 0.5 to 5.0 per cent and a silver halide developing agent.

WILLIAM H. WOOD.